

N. V. HYBINETTE.

PROCESS OF CIRCULATING SOLUTION FOR ELECTROLYSIS.

APPLICATION FILED JUNE 26, 1913.

1,128,315.

Patented Feb. 16 1915.



Witnesses:

B. Dommers

C. Leckert

Inventor:

Noak Victor Hybinette.

By Henry W. B. Atty.

# UNITED STATES PATENT OFFICE.

NOAK VICTOR HYBINETTE, OF CHRISTIANIA, NORWAY, ASSIGNEE TO PACIFIC SECURITIES COMPANY LIMITED, OF TORONTO, CANADA.

## PROCESS OF CIRCULATING SOLUTION FOR ELECTROLYSIS.

1,128,315.

Specification of Letters Patent.

Patented Feb. 16, 1915.

Original application filed June 5, 1912, Serial No. 701,780. Divided and this application filed June 26, 1913.  
Serial No. 775,955.

*To all whom it may concern:*

Be it known that I, NOAK VICTOR HYBINETTE, a subject of the King of Norway, residing at Christiania, Norway, have invented a Process of Circulating Solution for Electrolysis, of which the following is a specification, and is a division of my application, Serial No. 701,780, filed June 5, 1912.

This invention has for its object an improvement in a process of separating copper from nickel.

In a patent granted to me in U. S. A. November 28th 1905 under No. 805,969, I describe a process of refining copper nickel matte. A metallic copper nickel anode is electrolyzed in a bath of sulfate of nickel. The cathode is surrounded by a filtering bag and the electrolyte is circulated from cathode to anode through the said bag and then into a cementation tank where the copper absorbed from the anode is removed by cementation, whereupon the solution is again returned to the cathode side. However, even at its best the cementation is slow and costly and would be impracticable were it not that I have succeeded in devising means whereby the circulation in the plating tanks can be reduced very considerably and the amount of solution to be cemented is correspondingly diminished. The cost of cementation is namely in this case almost in direct proportion to the volume of solution and not to the amount of copper. The filter separating anode from cathode is so open that when the volume of circulation is reduced below a certain limit the filtering takes place only in that part of the filter that is nearest to the inlet for the fresh solution. When there is no filtering in the other parts of the filter diffusion sets in and ions of copper wander into the cathode compartment, contaminating the nickel. If for instance the electrodes are two feet wide by three feet deep and if the solution is run in

at the top at a slow rate it will soon be found that copper is entering at the bottom and contaminating that part of the cathode plate. If the flow of solution enters at the bottom the diffusion and contamination takes place at the top. I have now found that by alternatingly entering the flow of solution at the top and bottom, I can make a great saving in the amount of solution necessary to keep the copper outside of the filter.

In the annexed drawing is shown an electrolytic cell adapted for carrying out the process. Said cell is of a well known construction and need not here be described in its details.

A designates the cathode compartment, B the anode compartment, C and D pipes entering the cathode compartment, the pipe C having its lower end at the top of said compartment. The tops of these pipes are formed as funnels E, F, and into these funnels is supplied electrolyte through pipes G, H, said pipes being connected with a main supply pipe K through a two-way cock I. The cock is now alternately set in one or the other position and the nickel sulfate solution accordingly will be led alternately to the pipe C or to the pipe D.

What I claim is:—

In the process of separating copper from nickel by electrolysis and circulation through a filter from cathode to anode, the step which consists in passing the electrolyte alternately into the bottom and top of the cathode compartment thereby making it possible to reduce the quantity of solution to be circulated.

Signed at London, England, this 9th day of June 1913.

NOAK VICTOR HYBINETTE.

Witnesses:

H. D. JAMESON,

O. J. WORTH.